

## UNITED STATES PATENT OFFICE.

HENRY DREYFUS, OF LONDON, ENGLAND.

MANUFACTURE OF ARTIFICIAL SILK, ARTIFICIAL HORSEHAIR, AND THE LIKE.

No Drawing. Application filed June 28, 1923, Serial No. 648,350, and in Great Britain August 11, 1922.

This invention relates to the manufacture of artificial silk, artificial horsehair or like threads or filaments from solutions of cellulose acetate in particular, but applies also to their production from other solutions of esters of cellulose or of ethers of cellulose such as for example as ethyl-, methyl- or benzyl cellulose, or from mixtures of any of such cellulose derivatives, all of which solutions are 5 hereinafter included in the term cellulose derivative solutions. The invention solely concerns processes in which the artificial threads or filaments are produced by the dry or evaporative method of formation, that is 10 to say by extruding a solution of the cellulose derivative or derivatives in or containing a volatile or vaporizable solvent or solvents, through jets or spinnerets into a heated or other atmosphere in which the filaments or 15 threads solidify by evaporation of solvent. In particular the invention relates to the manufacture of threads, filaments or the like from cellulose acetate solutions, by dry or evaporative spinning.

20 In the manufacture of artificial threads or filaments from solutions of cellulose acetate or other cellulose esters or ethers such as referred to by the evaporative method, it is usual to employ spinning solutions of relatively low concentration, containing not more 25 than about 16 per cent of the cellulose derivative or derivatives in the solvent or solvents used.

It has now been found that by employing 30 for the dry or evaporative spinning solutions of substantially higher concentrations, containing not less than 20% and preferably not less than 25%, e. g., about 25 to 30% or more of the cellulose derivative or derivatives, and especially in the case of cellulose acetate solutions, artificial threads or filaments of improved quality can be obtained, possessing greater mechanical strength and rounder section, and showing much less tendency to crinkle or turn woolly in appearance under the action of very hot or boiling water, than is the case with dry-spun artificial threads or filaments, made from the less concentrated solutions previously employed. It is moreover 45 found that, especially in the case of cellulose acetate, the employment of solutions of high concentrations as referred to has the further advantage of obviating or greatly reducing what may be called "glitter" of the threads, 50 filaments or the like, that is to say, a glitter-

ing or scintillating effect which is sometimes possessed by filaments or threads formed by evaporative or dry spinning from solutions of the relatively low concentrations usually employed, and possibly due to the sectional 60 configuration of the filaments resulting from the spinning of such solutions, by the dry or evaporative method of formation. This "glitter" coated effect or glitter-producing structure of the filaments or the 65 like can in some cases be a disadvantage. For example, in cases where goods in hank, woven or knitted fabric or other form, made with threads showing such glitter effect are dyed in black or dark colours, it is 70 sometimes found that the dyed goods give an impression as if the artificial silk is dyed only partially or not deep enough or that they have a worn appearance, this being more especially seen in fabrics.

75 By forming the dry spun threads, filaments or the like from cellulose acetate solutions for example, of high concentrations such as before referred to, it will be seen that the filaments or threads are stronger than those made from solutions of the usual low concentrations, not so liable to crinkle or turn woolly as a result of the action of hot water, and moreover that "glitter" or glitter-producing structure is obviated or greatly reduced, 80 with its tendency to give on dyed goods, and especially goods dyed in black or dark colours, the appearance before referred to.

85 The following are two examples of spinning solutions which may be employed according to the invention, it being understood that these are given only by way of illustration and that other solvents or solvent mixtures may be employed and that the concentrations can be varied without departing 90 from the invention.

*Example 1.*

95 Cellulose acetate is dissolved in acetone in quantity to give a solution containing about 100 20 to 30 per cent, preferably about 25 to 30% cellulose acetate.

*Example 2.*

105 Cellulose acetate is dissolved in acetone containing about 5 to 10 per cent of alcohol and about 5 per cent of water, in a quantity to give a solution containing about 20 to 30 per cent, preferably about 25 to 30% of cellulose acetate in the solvent mixture.

The solutions are dry spun in the known way by extrusion through spinnerets into a heated atmosphere.

While my invention relates especially to the manufacture of artificial threads, filaments or the like from cellulose acetate solutions by the dry or evaporative method it is also applicable to their production by the dry or evaporative method from solutions of other cellulose esters or ethers or mixtures of cellulose esters or/and ethers.

What I claim and desire to secure by Letters Patent is:—

1. Process for the manufacture of artificial filaments and threads, characterized in that the same are dry spun from concentrated so-

lutions of organic substitution derivatives of cellulose containing not less than 25 per cent of cellulose derivative.

2. Process for the manufacture of artificial filaments and threads, characterized in that the same are dry spun from concentrated cellulose acetate solutions containing not less than 25 per cent of cellulose acetate.

3. Process for the manufacture of artificial filaments and threads, characterized in that the same are dry spun from solutions of cellulose acetate containing 25 to about 30 per cent of cellulose acetate.

In testimony whereof I have hereunto subscribed my name.

HENRY DREYFUS.